

Nov. 2, 1965

D. D. BROWN ET AL.

3,214,961

## METHOD AND APPARATUS FOR TESTING ELASTOMERIC SEALANTS

Filed Oct. 1, 1963



INVENTOR.  
DELMONT D. BROWN  
JAMES H. PAX

BY: Margell, Johnston, Cook & Post  
ATT'YS

1

3,214,961

**METHOD AND APPARATUS FOR TESTING  
ELASTOMERIC SEALANTS**

Delmont D. Brown, North Baltimore, and James H. Pax,  
Rudolph, Ohio, assignors to The D. S. Brown Company,  
North Baltimore, Ohio, a corporation of Ohio

Filed Oct. 1, 1963, Ser. No. 312,976

12 Claims. (Cl. 73—15.6)

This invention, in general, relates to testing machines and methods and, more particularly, pertains to machines and methods useful in the testing of weather-sealing properties of elastomer compositions under varying temperatures and stresses. The testing machines and methods of the invention are particularly adapted for the testing of elastomer strips and caulk-type joint sealants under conditions simulating field conditions wherein said strips are employed to seal any type of expansion and compression joint.

Considerable attention has been given in recent years to the use of compressible strips of elastomer as seal strips in concrete joints of highways and bridges. These compressible, resilient strips are used to seal highway and bridge expansion and contraction joints against intrusion of water, dirt and the like into the expansion joints. The strips compress and expand as the expansion and contraction joint expands and contracts under variable climatic temperature conditions. Semisolid, caulk-type joint seals include the known asphalt or asphalt-elastomer mixtures used to seal expansion and contraction joints as well as other caulking compositions. Caulk-type joint seals are discussed more fully later in the specification.

The testing machines of the invention may be employed to test or screen various elastomer compositions in terms of their potential properties as sealing strips in joints of highways, buildings, airstrips, bridges, sidewalks and the like. The machines of the invention and the strip-compressing components thereof are constructed in a manner whereby the elastomer compositions can be subjected to conditions of approximate maximum compression of the strips anticipated in their ultimate use as highway seal strips at hot and cold temperatures. One of the properties of the strips which is determined is that of elastic recovery of the strip after it has been subjected to maximum anticipated compression at hot and cold temperatures in accord with the test procedures hereafter described.

Briefly, the test machines of the invention and the strip-compression apparatus used therewith comprises a fixed block and a movable block. The movable block is movable toward and away from the fixed block. An elastomer strip is inserted and held between adjacent faces of the two blocks.

The fixed block is fixedly, but preferably removably, attached to the frame of the machine. The movable block is fixedly, but preferably removably, attached to a movable element or plate of the machine which, in turn, is reciprocally movable by power-operated means toward and away from the fixed block at a slow rate of motion.

Alternatively, both blocks may be reciprocally mounted on the machine frame, and both blocks may be driven to provide the relative reciprocal motion of said blocks toward and away from each other to compress and decompress the elastomer strip therebetween.

In accordance with a preferred embodiment of the invention, the two blocks with an elastomer strip compressed therebetween may be held together as a unit by a supplemental frame structure attached to the blocks after the strip has been compressed by the machine or the frame to the desired state of compression. The two blocks and the supplemental frame structure may then be removed as a unit from the machine and placed in a hot or cold

2

chamber wherein the strip in the compressed state is subjected to the desired test temperature or temperatures.

The upper, adjacent corners of the test blocks preferably are cut away so as to form depressions when the blocks are juxtaposed with a strip compressed therebetween. This depression is adapted to hold a test liquid such as an antifreeze liquid, e.g., a mixture of water and ethylene glycol. After the strip has been subjected under compression to the hot and/or cold temperature test conditions, the blocks are slowly moved apart, e.g., by retracting the movable block away from the fixed block. When the liquid in the depression begins to leak through between the joint between the sides of the elastomer strip and the contacting face of the test block or blocks, the distance between the blocks is measured. This test measures the point at which the elastic strip loses its sealing function in relation to the side walls of the test blocks.

An embodiment of a test machine of the invention is illustrated in the drawings wherein:

20 FIG. 1 is a perspective view thereof;  
FIG. 2 is a cross-section taken on section 2—2 of FIG. 1;

25 FIG. 3 is a perspective view of a test block and frame assembly thereon which may be used in a portion of the test procedures of the invention;

FIG. 4 is a transverse cross-section of the test blocks at the seal leakage stage of the test procedures; and

FIG. 5 is a schematic view of a hydraulic drive for the movable plate and block.

30 Referring to the drawing, which illustrates a preferred embodiment of the invention, there is shown a flat frame plate 1. A pair of frame blocks 2, 3 are bolted by the bolts 4 to the frame plate 1 along opposite edges thereof. The frame blocks 2, 3 are parallel and contain in their 35 inward, opposing faces grooves 5, 6. The grooves 5, 6 form slide tracks for a movable plate carrying the movable testing block, hereafter described.

35 In addition to the frame plate 1 and frame blocks 2, 3, the machine frame further comprises a pair of parallel frame bars 7, 8 attached to the frame plate 1 by bolts 4. These frame bars 7, 8 are parallel and extend across one end of the frame plate 1 transversely to the frame blocks 2, 3. The frame bars 7, 8 function as journal bars for the mechanical drive hereafter described and may also support 40 a gear reducer 9 fixedly mounted on the top edges thereof at one corner of the machine. The gear reducer may be mounted at other positions, if desired. The gear reducer 9 is driven by an electric motor (not shown). The output shaft of the gear reducer has mounted thereon a drive 45 sprocket 10. The drive sprocket 10 drives via the chain 11 a larger sprocket 12 mounted on the gear shaft 13 of the spur gear 14. The gear shaft 13 is rotatably journaled in the frame bars 7, 8.

45 The spur gear 14 rotatably drives the idler gears 15, 16, which, in turn, rotatably drive the gears 17, 18. The gear shafts 25 of idler gears 15, 16 are rotatably journaled in the frame bars 7, 8. Gears 17, 18 have threaded axial, apertures threadedly engaged with the machine screw threads 21 of rods 19, 20, respectively, 50 the ends 19' and 20' of which axially slidably are supported in holes in frame bar 8. One end of rods 19, 20 is fixedly held by nuts 22 in tapped holes 24 in the edge of the movable plate 23 whereby the rods are non-rotatable. The movable plate 23 is slidably mounted in the opposing grooves 5, 6 of the frame blocks 2, 3.

55 The plate 23 is reciprocated in the grooves 5, 6 by rotatably turning the gears 17, 18 by means of the gear and chain-sprocket drive heretofore described. When the chain-sprocket drive is activated, the gears 17, 18 are rotated at equal, slow rates of rotation. As the gears rotate, the threaded engagement thereof with the

machine screw rods 19, 20 causes the rods and the movable plate 23 to move in one direction or the other, depending upon the direction of rotation of the gears 17, 18. Control means for selecting the direction of rotation of the gears 17, 18 may be any conventional means, the simplest and most expedient being reversible electric motor (not shown) for driving the gear reducer 9.

A test block 26, e.g., a concrete block, is fixedly but removably attached to the movable plate 23 by means of bolts 27 extending through the block 26, a cross plate 28, and a synthetic rubber pad 29, e.g., silicone rubber, and threaded secured in the movable plate 23. The test block 26 is thus reciprocally movable with the movable plate 23. The rubber pad 29 spreads the force of bolts 27 and prevents accidental breakage of the concrete blocks when the bolts are tightened.

The fixed block structure of the test machine comprises a fixed plate 30 fixedly attached to and extending across the end of the frame plate 1 between the frame blocks 2, 3. The stationary test block 31, e.g., a concrete block, is fixedly attached to fixed plate 30 by means of bolts 32 extending through the test block 31, a cross plate 33 and a synthetic rubber pad 34. The bolts 32 are threaded in tapped holes in the fixed plate 30 and/or the frame plate 1. Fixed plate 30 may be supported in the grooves 5 and 6 and fixedly attached to frame blocks 2, 3 by bolts, welding, etc. The fixed plate 30 and movable plate 23 are spaced from base plate 1 sufficiently to allow a shallow pan P to be placed beneath the plates, the shallow pan being used to collect liquid leakage in the test procedures hereafter described. Instead of a shallow pan, a liquid sensing device may be used, e.g., one with an electrical circuit including a timer, motor-deactivating switch, or alarm device and a sensor element activating the circuit when the first drop of liquid falls through the test joint with the seal therein.

The contiguous, upper corners of the test blocks 26, 31 have cut away segments 35, 36 forming a depression 37, e.g., an oval depression, when the blocks are juxtaposed with the elastomer strip 39 under test compressed therebetween. The elastomer strip is inserted between the blocks in a manner whereby the strip substantially follows the contour of the juxtaposed upper surfaces of the blocks 26, 31. It is preferably held in the space 38 between the blocks at a distance slightly below, e.g.,  $\frac{1}{8}$ ", below the upper surface of the juxtaposed blocks.

The test blocks 26, 31 have in their opposite sides inwardly-directed slots or grooves 40, 41. These slots or grooves accommodate the shanks 42 of bolts 43 having on their threaded ends a threaded nut, e.g., the wingnuts 44. The shanks 42 of the bolts extend through bars or plates 45, 46 positioned across opposite ends of the test block assembly (FIG. 3). The bolts and bars or plates 45, 46 form frame assembly which can be attached to the test block assembly on the machine when the elastomer strip is compressed between the test blocks 26, 31. By tightening the bars or plates 45, 46 against the ends of the test blocks, the test block assembly with the resilient strip compressed therebetween can be locked in the frame assembly. The test block assembly can then be removed from the machine by removing bolts 27, 32. The four holes 47, shown in the test block assembly of FIG. 3, are the holes in the test blocks 26, 31 through which said bolts extend.

The mechanical drive for moving the movable plate and movable block thereon preferably is powered by a reversible, variable speed electric motor. The rate of movement of the movable test block can thus be controlled by control of the rate of revolution of the motor. A constant output speed motor may be used, however, if desired. Furthermore, the mechanical drive may be replaced by a metal bar or bars attached at one end to the machine frame and at the other end to the movable

plate 23. The metal bar or bars are made of a metal or metal alloy which expands and contracts linearly under increasing and decreasing temperatures, respectively. The length of the bars and the linear coefficient of expansion of the metal or metal alloy determines the amount of movement of the movable plate between the temperature extremes of the test. In these adaptations of the invention, the test machine itself is placed in the freezing chamber and/or heating oven employed in the test procedure in order to expand or contract the metal bars or bellows while at the same time subjecting the elastic strip to the test temperature. The thermally expandable and contractable metal bars may be operatively associated with both blocks, instead of only one block, in test machines wherein both of blocks 26, 31 are mounted on the frame, e.g., by also mounting block 31 on movable slide plate like plate 23, for relative reciprocal motion toward each other at increasing temperatures and away from each other at decreasing temperatures.

Another alternate form which can be substituted for the mechanical drives for the movable plate and block is a hydraulic fluid system comprising a conventional hydraulic chamber fixedly mounted on the machine frame with a movable piston therein. The piston rod is connected to the movable plate. The piston and piston rod are moved in either direction at the desired linear rate of hydraulic force applied against the appropriate side of the piston.

A hydraulic drive is illustrated schematically in FIG. 5. The over-all test machine structure may be substantially the same as the test machine embodiment of FIGS. 1 and 2 with the mechanical drive and associated support parts therefor omitted. The movable plate 23 with movable block 26 thereon are driven by a hydraulic system comprising a hydraulic fluid chamber 50 with a piston 51 longitudinally reciprocable therein. The piston rod 52 of piston 51 is attached to the movable plate 23.

A pair of hydraulic fluid lines 53, 54 communicate the chamber 50 on each side of the piston 51 with opposite sides of the piston 56 of master hydraulic fluid cylinder 57. One of the lines 53, 54 has a bleed valve 55 which can be adjusted to control the rate of flow of hydraulic fluid between the master cylinder and the hydraulic chamber 50 to give the desired rate of linear movement to plate 23. The piston 56 may have a single piston rod 58 which is movable in either direction by mechanical power, e.g., a rack and pinion. The pinion may be driven by a reversible motor through slip clutch to allow slip in the mechanical drive when the bleed valve is adjusted to allow lesser volume movement of hydraulic fluid than the movement provided by operation with the clutch at minimum slip and avoid overload in the hydraulic pressure. Alternatively, the piston 56 may also have a second, oppositely directed piston rod 59, each of which piston rods 58, 59 coupled to a power source, moving the respective rods in opposite directions. An example of the latter is coil tension springs 60, 61 attached to each rod with multiple advantage mechanism, a ratchet and pawl mechanism of the automobile bumper jack type for individually and manually tensioning each spring. Each spring in the untensioned state should have sufficient sag so as not to become tensed while the other spring is moving the piston 56. The hydraulic fluid should be one having good fluid properties at cold temperatures, e.g., in the range of the 0° F. to -65° F. temperatures used in the test procedures herein described.

The movement of the test blocks toward each other in the heating or aging cycle of the test is not of great or critical importance, however. The oven treatment is primarily an accelerated aging treatment of the elastomer seal strip, and it can be done with the strip held in the previously described frame assembly to conserve space in the oven. Before allowing the aged seal strip to expand, it is taken down to the cold test temperature. The prime purpose of this type of test is the collection of

data on cold flexibility movement or resilience of the rubber in cold temperatures, compression and permanent set due to the aging, and the determination of positive sealing by having a liquid on top of the seal utilizing the actual, finished seal.

When testing elastomer strips as highway or bridge concrete joint seals, the test blocks 26, 31 preferably are concrete blocks so that the surfaces of the blocks which contact the elastomer strips are comparable texture to concrete highway or bridge sections. Where the strips being tested are intended for use as sealing strips or gaskets between other types of surfaces, other materials may be selected as the test blocks. Where relatively smooth surfaces are involved, metal blocks or the like may be used.

#### Testing methods

Elastomer seal strips, as a general rule, are most critically adversely affected in terms of their elastic recovery or resilience upon lateral expansion of the strip at cold temperatures. The strips have a poorer elastic recovery from compression when cold than when warm. Accordingly, the test procedures herein set forth are made with the objective of testing the strips by simulating the actual or anticipated field conditions at which the sealing function of strip usually breaks down.

As an example of an actual field condition for a highway in which the expansion and contraction joints are sealed or to be sealed by the elastomer strip under test, assume a warm, sunny winter day in which the concrete sections are warmed by both the warm air and by radiation heat of the sun. The joints are well contracted under this condition. There is a sudden temperature drop in late afternoon or early evening to a temperature in the range of 0° F. to -65° F. The elastomer strips become cold quickly, and the highway sections cool and contract. The joints begin to open, and the cold elastomer strips must expand laterally to maintain the seal between the side walls of the strips and the side walls of the joints. This is a critical area in which the strip must expand laterally under most adverse conditions in terms of its lateral elastic recovery.

The tests hereafter described simulate such conditions and preferably are even somewhat more severe than would be the worst anticipated field condition. The collection of data on the sealing qualities of the strip with lateral expansion of the strip at the selected cold test condition preferably is made first on the strip before it is subjected to aging by heat. The strip is then aged at high temperature in an oven with the strip under about maximum anticipated compression. The oven temperature is ordinarily above maximum anticipated field temperature in order to accelerate the elastomer aging process and shorten the total test time. The reason why the strip is compressed at about maximum anticipated compression during the aging step is that in field use the strip would be under the same conditions when it is at its highest temperature, the joints being contracted or closed the greatest amount when the highway concrete sections are the hottest. Our test methods, however, can be used, though not as effectively in terms of duplication of field conditions for measuring the effect of permanent set due to heat aging of the elastomer, with the aging done at substantially less than maximum anticipated compression.

After the heat aging step, the strip is tested again at the cold temperature by the cold temperature procedure previously described. By comparing the data obtained both prior to and after aging for percent of recovery of the original width of the strip under cold temperature lateral expansion of the strip as the test machine joint expands up to the point of loss of seal against liquid penetration, the effect of aging on the strip can be measured. This data can be very helpful in future research to find modified or new compounding measures for vulcanizable elastomer compositions and/or modification of the physi-

cal structures of the strips to improve the over-all quality of the strips.

The testing of the suitability of a particular elastomer strip as a concrete joint seal or the like is conducted on 5 the machine illustrated in the drawings by the following procedure.

The blocks 26, 31 are separated enough to insert the elastomer strip 39 therebetween with the upper surface of the strip substantially flush with or slightly below the 10 contour of the adjacent, upper surfaces of the blocks. The movable plate 23 and block 26 are moved toward the block 31 by the mechanical drive system of the machine until the strip 39 is compressed to about the maximum amount of compression anticipated in field use. 15 At this stage, the frame assembly shown in FIG. 3 may be assembled and tightened about the test blocks. The bolts 27, 32 then may be removed, and the test block and frame assembly thereabout are lifted from the test machine, the elastomer strip 39 still being in the state of 20 maximum anticipated compression. As an alternative, the entire test machine (preferably excluding the electric motor) may be used in this portion of the test, and the steps of frame assembly and removal of the test blocks may be omitted.

25 The test machine or the test block-frame assembly, as the case may be, is brought to a subfreezing temperature in the range of about 0° F. to -65° F. in order to subject the compressed strip to a selected, subfreezing temperature for a period of about 18-72 hours in a cold box, 30 refrigerated chamber or room, etc.

Then a liquid which will not freeze at the test temperature is placed in the depression 37. A mixture such as a 50-50 mixture of water and ethylene glycol may be used, for example. Preferably in the cold box, refrigerated chamber or room, etc., and in any case without allowing appreciable warming of the cold test blocks and elastomer strips above the subfreezing temperature to which the elastomer seal strip is subjected and with the 35 blocks 26, 31 remounted on the machine (if removed for the cold temperature segment of the test), the mechanical drive is activated to move slowly the movable block 26 away from the fixed block 31. A linear movement of about  $\frac{1}{16}$ " to  $\frac{1}{2}$ " per hour, in most cases about  $\frac{1}{16}$ " to  $\frac{3}{8}$ " per hour, may be selected. The movement 40 is stopped when the liquid L in the depression 37 begins to leak between the contacting wall or walls of test blocks 26, 31 and the strip 39 (FIG. 4). The distance between the blocks 26, 31 is measured to ascertain the degree of elastic recovery of the elastomer strip up to the 45 point where its liquid-tight seal with the test blocks is lost.

The same strip is then again compressed to the smallest width anticipated in actual service. The frame assembly (FIG. 3) is assembled and tightened about the test 50 blocks, and the test block-frame assembly is removed from the machine. The removed unit, with the elastomer seal strip under compression, is placed in a heating chamber or oven for an accelerated aging of the elastomer. The aging temperature may be a selected temperature in the range of 150-230° F., and the selected aging time 55 may be in the range of 48-120 hours.

After the accelerated aging step, the unit is placed, with the strip 39 still in its compressed state, in a refrigerated room or chamber wherein the subfreezing temperature portion of the test, above described, is repeated 60 at a temperature and time in the ranges above stated. With the test blocks remounted on the test machine in the cold box, refrigerated chamber or room, etc., the liquid L is poured into the depression 37, and the block 26 is retracted slowly away from block 31 until leakage 65 between the test block or blocks and the elastomer seal strip is noted at the cold temperature of the test.

As an alternative test procedure after the accelerated aging, a dynamic type test procedure can be used wherein 70 the machine with the test blocks thereon and the liquid L

always in the depression can be moved to a cold atmosphere (0° to -65° F.) then to a hot atmosphere (95-140° F.), and then back to the cold atmosphere. The elastomer seal strip is given the calculated or anticipated maximum and minimum compression or expansion between the test blocks in the two respective atmospheres. The leakage of the seal is ascertained at the critical stage, i.e., in the cold atmosphere, as aforescribed.

By conducting the foregoing tests on a number of different types of elastomer compositions and/or structural styles of elastomer seal strips, and by measuring for each seal strip tested its initial, uncompressed width, compressed width, time and temperature of the oven aging and subfreezing steps, rate of separation of the test blocks, distance between blocks at the first sign of a leak between the seal and the test blocks, and width of the seal after it is released from compression (a) immediately, (b) after 30-60 minutes at room temperature and (c) after 24 hours at room temperature, a compilation of data is assembled from which the better-performing elastomer strip or strips can be selected for further laboratory tests or field study.

As a specific example, with neoprene seal strips for concrete highway expansion joints, the test procedure above described was conducted at a subfreezing temperature of -30° F. for 22 hours, at a rate of separation of the test blocks of  $\frac{1}{16}$ " per hour, and at an aging temperature of 212° F. for 70 hours. The seal strip in the cold temperature expansion at -30° F. recovered 90% of its original width before leakage was detected. A lesser recovery was experienced upon cold temperature expansion after aging.

The machine and test procedures aforescribed may also be used to ascertain the sealing properties of caulk-type, semi-solid, expansion and contraction joint seals for highways, bridges, buildings, airstrips, etc. A well known caulk-type, highway seal is the asphalt seal made by pouring hot, liquid asphalt into the joint. Upon cooling, the asphalt becomes a semi-solid mass with cold flow properties. Similar semi-solid seals are made with mixtures of asphalt and elastomers such as natural rubber or synthetic elastomers (e.g., butyl rubber, butadiene-styrene copolymers, neoprene, etc.). The elastomers improve the flexibility and resilience of the asphaltic-type seal.

The caulk-type, semi-solid seals behave somewhat differently from the elastomer seals heretofore discussed in that they have little or essentially no elastic resilience when compressed. The caulk-type seal relies upon adhesion of the caulking composition to the side walls of the joint to maintain the seal as the expansion and contraction joint opens. In theory, the seal is stretched as the joint opens in cold weather and returns to the normal state as the joint contracts in hot weather. In practice, however, the caulking seal usually either pulls away from the one or both of the side walls of the joint or cracks down the middle. These cracks in the seals themselves or between the seal and the side walls of the joints fill with highway dirt and other solids, reducing the compressibility of the caulking seal. The ultimate result of build up of such solids in the cracks, if left uncorrected, is a joint seal filled with enough incompressible solids so that the seal will not compress enough in hot weather, as the concrete highway sections or the like expand, to take up the expansion. Pressures in the concrete sections develop sufficient magnitude to cause the concrete to break. Another adverse effect is known as roping, which is a problem with caulking seals such as polysulfide rubber caulking seals.

It will be apparent, therefore, that laboratory testing of caulking-type seals, as well as the laboratory testing of elastomer, dry-type seals heretofore discussed, is of practical value. The tests are conducted by essentially the same procedure as the cold temperature (0° F. to -65° F.) test. Aging of the seal at high temperature, of course, has no purpose with asphalt-type seals, but the

seal may be subjected to and/or tested at high temperatures (e.g., 100-140° F.) if desired.

As an example of a testing procedure with a caulking-type seal, hot asphalt is poured into a joint between concrete blocks 26, 31 with the joints spaced apart at the smallest, anticipated spacing between concrete sections of a highway or bridge joint. The test machine is placed in a cold box, refrigerated room, etc., maintained at a preselected temperature in the range of 0° F. to -65° F., e.g., -30° F. When the concrete blocks and seal are at equilibrium with the cold atmosphere, the test machine is activated. Prior thereto, antifreeze liquid L is placed in the depression 37. Movable block 26 moves away from block 31 at a slow, predetermined rate. When the liquid seeps through the seal, the test is stopped. The spacing between the concrete blocks at the point of loss of liquid seal is recorded. Other observations of value which can be made during the test are notations as to surface cracks formed in the seal as the joint expands, cause of loss of liquid seal (e.g., separation of a wall or walls of the concrete block and the caulking seal or a break in the middle of the seal), and like data which will be of value in future research for improving performance of the seal.

Thus, the test machines and test methods herein defined provided dynamic test conditions simulating field use of elastomer strips as joint seals between expanding and contracting sections. Considerable time and expense can be saved by the employment thereof in screening and evaluating various elastomer compositions and/or various elastomer strip structural styles for a given field use. Similar, valuable, experimental data can be obtained in tests with caulk-type, semi-solid seals.

The invention is hereby claimed as follows:

1. A testing machine comprising a frame, a first block and a second block mounted on said frame, means on said frame mounting said blocks for relative, horizontal reciprocal movement toward and away from each other, and means for providing slow, reciprocal, relative movement between said blocks toward and away from each other to compress and decompress, respectively, an elastomer strip between adjacent faces of said blocks, the upper surfaces of said blocks being recessed to form a liquid-receiving depression in said upper surfaces with said strip compressed between said blocks at said depression.

2. A testing machine as claimed in claim 1 wherein said blocks are concrete blocks.

3. A testing machine comprising a frame including a pair of spaced, parallel frame members, horizontal slide means on said frame members, a first block mounted on said frame and extending between said frame members, a plate extending between said frame members and slidable on said slide means toward and away from said first block, a second block mounted on said plate, and mechanical drive means coupled to said plate for moving said plate and second block at a slow linear speed away from said first block, the upper surfaces of said blocks being recessed to form a liquid-receiving depression in said upper surfaces with said strip compressed between said blocks in said depression.

4. A machine as claimed in claim 3 wherein said mechanical drive means includes a threaded rod fixedly attached to said movable plate, and a rotatable drive member threadedly engaged with said rod.

5. A machine as claimed in claim 3 wherein said blocks have aligned grooves in opposite side walls of each of said blocks, said grooves adapted to receive members of a frame assembly adapted to be used to clamp said blocks together with an elastomer strip compressed therebetween, means releasably attaching said first block to said frame, and means releasably attaching said second block to said movable plate.

6. An assembly used in testing properties of elastomer strips comprising a first concrete block, a second concrete block, an elastomer strip compressed between opposing faces of said blocks, and a frame assembly about

said blocks holding said blocks together with said strip compressed therebetween, the upper surfaces of said blocks being recessed to form a liquid-receiving depression in said upper surfaces with said strip compressed between said blocks in said depression.

7. A testing machine comprising a frame including a pair of spaced, parallel, frame members, horizontal slide means on said frame members, a first block mounted on said frame and extending between said frame members, a plate extending between said frame members and slidably on said slide means toward and away from said first block, a second block mounted on said plate, and fluid-driven drive means coupled to said plate for moving said plate and second block at a slow linear speed away from said first block, the upper surfaces of said blocks being recessed to form a liquid-receiving depression in said upper surfaces with said strip compressed between said blocks in said depression.

8. A process for testing the joint sealing properties of elastomer seal strips which comprises compressing between a pair of compression members an elastomer strip, subjecting said elastomer strip in the compressed state to a subfreezing temperature, forming a pool of liquid, which does not freeze at said subfreezing temperature, above and in contact with the joints between the sides of said compressed strip and said compression members, slowly decompressing said strip at a subfreezing temperature by slowly separating said members until liquid from said liquid pool seeps through one of said joints, and measuring the spacing between said compression members when said liquid seeps therethrough.

9. A process for testing the joint sealing properties of elastomer seal strips which comprises compressing an elastomer strip between a pair of compression members, aging said strip in the compressed state in an oven at an elevated temperature, subjecting said strip in the compressed state to a subfreezing temperature, forming a pool of liq-

uid, which does not freeze at said subfreezing temperature, above and in contact with the joints between the sides of said compressed strip and said compression members, slowly decompressing said strip at a subfreezing temperature by slowly separating said members until liquid from said liquid pool seeps through one of said joints, and measuring the spacing between said compression members when said liquid seeps therethrough.

10. A process as claimed in claim 8 wherein said subfreezing temperature is in the range of 0° F. to -65° F.

11. A process as claimed in claim 9 wherein said subfreezing temperature is in the range of 0° F. to -65° F., and said elevated temperature is in the range of 150-230° F.

15. 12. A process for testing the joint sealing properties of semi-solid, caulking seals which comprises forming a semi-solid, caulking seal between a pair of closely spaced members, subjecting said members and seal to a subfreezing temperature, forming a pool of liquid, which does not freeze at said subfreezing temperature, above and in contact with the joints between said seal and said members, slowly widening the space between said members at a subfreezing temperature until liquid from said liquid pool seeps through the seal formed between said members by said semi-solid, caulking seal, and measuring the spacing between said compression members when said liquid seeps therethrough.

#### References Cited by the Examiner

##### UNITED STATES PATENTS

|           |       |        |       |         |
|-----------|-------|--------|-------|---------|
| 2,283,743 | 3/42  | Lessig | ----- | 73—91 X |
| 2,933,921 | 4/60  | Gloor  | ----- | 73—93   |
| 3,062,009 | 11/62 | Thiele | ----- | 73—92 X |

35 RICHARD C. QUEISSE, *Primary Examiner.*

DAVID SCHONBERG, *Examiner.*